

## UNITED STATES PATENT OFFICE.

PETER JUNG, OF BERLIN-NEUKOLLN, GERMANY.

## PROCESS OF MAKING BRIQUETTES.

No Drawing. Application filed July 28, 1922, Serial No. 578,262, and in Germany May 24, 1921.

This invention relates to a new or improved process for the production of briquettes from bituminous or carbonaceous and like materials, as for example, small coal, lignite, peat and the like.

Heretofore, briquetting processes may be said to have been divided into two principal classes. In one of these, there was added to the material a binder medium of an entirely different nature, as for example, cement, plaster of Paris, and the like. In the other of these classes there was added to the material a binder having a composition similar to that of the material to be briquetted, or the binder medium was formed by special treatment of the bituminous substances in the raw material itself. For example, pitch, naphthalene, and the like have been added as binders, or binding mediums have been produced in the raw material itself as by means of the heat and pressure used in carrying out the briquetting process.

The process according to the present invention differs essentially from those practised heretofore, and is distinguished by effecting a change in the physical condition of the material to be briquetted and using this physically changed material as a binding medium. In this, the invention is distinguished from the known processes in which bituminous and like binders are added to the material, and from the known processes in which bituminous and like constituents of the raw material are influenced by pressure and heat conditions of the briquetting process so that they function as binders.

According to this invention, a portion of the raw material to be briquetted, or a predetermined quantity of a similar material, is ground to colloidal fineness in water and is thoroughly mixed with a suitable amount of the raw material to be briquetted. It has been found that in the briquetting of such a mixture, only relatively low pressures are necessary for the production of quite firm and hard briquettes. The portion ground to colloidal fineness as aforesaid, acts as a very efficient binder and the briquettes produced with even relatively low pressure satisfy all technical requirements. The nature of the actions or reactions taking place during the process can only be presumed but it is not at all improbable that the colloidal slimes of the very finely ground material are very diffusely distributed and fill up all

interstices of the mass of material to be briquetted so that cohesion is increased to such a degree as to produce firm hard blocks as aforesaid.

It is not necessary for the purposes of this invention that the colloidally ground material should be the same as the raw material forming the principal constituent of the briquettes, as it may be advantageous to choose for the purpose such material as will give the best yield of colloidal medium and furnish the best results.

In addition to facilitating the production of firm hard blocks, the invention also presents a further advantage which will now be referred to. It has been found that materials which only dry with great difficulty when briquetted in the ordinary way will give up their water or moisture content with in an essentially shorter period when briquetted in accordance with this invention. This is a quite unlooked for result and is especially striking when using peat for the manufacture of the briquettes. For example, raw peat is taken containing anything up to 90% of moisture and the moisture contact is reduced by suitable means, and without experiencing any technical difficulty, to 60-70% and if the raw material is then briquetted with the addition of, say, 6% (calculated upon the basis of dry peat) of peat slime produced by grinding to colloidal fineness, the briquettes will lose so much moisture during the pressing operation and during a few days in stacks or heaps that the moisture content will be reduced to 20-25%. On the other hand, it is known to be a fact that the same reduction of moisture in raw peat, when the latter is dried in the usual manner in the open air, requires several months. This is a surprising result which cannot be accounted for theoretically. As a further example, brown coal, wet from the pit, can be directly briquetted in a similar manner.

The new or improved process, therefore, possesses great simplicity and is very economical in view of the fact that high pressures and high temperatures are not required. Also, it possesses the advantage, in common with other processes involving the addition of organic binders, that no increase in the content of ashes is necessary owing to the addition of binder mediums of a different kind. Upon the nature of the ma-

- terial to be agglomerated, that is to say the degree of ease or difficulty with which it lends itself to agglomeration, depends the question whether or not other materials can be mixed with it for agglomeration. For example, in the case of raw materials which readily lend themselves to agglomeration or binding, it is possible to mix with them substances or materials which in themselves 10 lessen or tend to lessen the agglomerative capacity of the mass. As an instance, a mass of peat to be agglomerated can have a higher percentage of coke waste or small coke added to it in admixture than heretofore.
- 15 Also, brown coal or lignite can have added to it in admixture nuts or knobs of brown coal which have been previously separated from it by sifting or riddling, which nuts or knobs have heretofore presented difficulties 20 in attempts to agglomerate or bind them in briquettes. It has been found that these admixtures, in many cases, facilitate the reduction of the moisture content of the briquettes not solely on account of the smaller 25 water content of the added materials but also on account of their influence on the internal structure of the block.
- Briquettes produced in accordance with this process are suitable for all general heating purposes and also for the purposes of 30 gasification and distillation, according to the materials employed for their composition.
- In order to enable the invention to be more 35 readily understood, the practical carrying out of one process will now be given by way of example.
- Assume the raw material to consist of raw peat which is equalized or made uniform in 40 known manner and contains 90% of moisture. As a first step, this moisture content may be readily reduced to 60% by the use of presses of known construction. A portion of this peat with reduced moisture content 45 is now ground with water in suitable grinders to such a degree of fineness that a completely even and smooth slime is obtained which, practically speaking, represents matter in permanent suspension. The mass of 50 raw material to be agglomerated may now be composed so as to consist of 79 parts of peat and 15 parts of small coke or waste coke. To this mass of mixture is now added a quantity of the slime equal to about 6 parts 55 calculated on the basis of the dry peat, and this slime is diffusely distributed in the mass so as to form an uniform mixture by the aid of any suitable mixing machine. The mass is now employed for the making of briquettes in briquette presses and a slight heating of the moulds of these presses during the 60 pressing may be beneficial. This heating may be done by exhaust steam from an engine.
- 65 Briquettes, made in accordance with the foregoing example, are delivered from the press containing approximately 35% of moisture and, if stored in sheds in single layers, the percentage of moisture will be further reduced by evaporation to 20-25% 70 within the space of 36 to 48 hours. Of course, this supplementary drying can be forced or hastened, provided that heated air is available, in the event of immediate shipment of the briquettes being essential. With 75 such supplementary or accelerated drying, the briquettes may be dried down to a moisture content of 25-30% of moisture within a few hours.
- Owing to the high content of oxygen in 80 briquettes made in this way, particularly briquettes made of mixtures, they require little air for combustion, they ignite easily and give off gas uniformly and easily. By admixture of suitably chosen raw materials, 85 briquettes can be obtained of graded calorific value, within possible limits.
- It has already been mentioned that briquettes produced by the improved process may 90 be very advantageously made use of for coking purposes. In proportion, as the constituents themselves are capable of being coked, lump coke is obtained suitable for use in furnaces. However, in the case of raw materials which of themselves would not produce any 95 concrete coke capable of withstanding pressure, no such coke could be produced by this process.
- Nevertheless, it has been proved that the 100 present process is exceedingly advantageous in combination with those known processes by means of which lump coke is obtained from raw materials which do not coke by themselves. For example, it has been suggested to add to brown coal such substances 10 as will act as fluxes during coking, including boric acid, clay or earth silicates, alkali compounds and so on, in order to produce a certain degree of sintering. In practising the present invention it has been found that 11 such sintering processes are carried out much more favourably that is to say with less addition of such materials as have been referred to, if the raw materials which are to be converted into lump coke are first briquetted in accordance with the process above 11 described and if the fluxes are added to the colloidal slime binding medium as well as such materials as are required to give off carbon during coking, such as highly molecular tar oils, tar residues and the like. In such slimes to be employed as binding media, therefore, there would be contained for example, small quantities of boric acid and tar in fine distribution. By this means a 12 firm smelting coke capable of withstanding pressure and suitable for smelting furnace work can be produced, for example, from brown coal, lignite, peat and the like.

I claim:—

1. A fuel in the form of a pressed mass, of a size suitable as a briquette, the same containing a large proportion of a solid fuel together with a small amount of solid fuel  
5 material ground to a substantially colloidal state of fineness and capable of forming a substantially permanent suspension in wa-  
ter, the colloidal fuel being uniformly dis-  
tributed throughout the said mass, and being  
10 in addition to any naturally occurring col-  
loidal material in such fuel.

2. A process for briquetting coal, lignite, peat and like materials which comprises grinding at least one of such materials in  
15 water to such a condition of fineness that originally-noncolloidal solid parts thereof assume the condition of a colloidal disper-  
sion and substantially permanent suspen-  
sion, and thereafter mixing a quantity of  
20 said so formed colloidal dispersion with a quantity of the carbonaceous material to be

briquetted in such proportions as to enable it to be molded into briquettes.

3. The process for briquetting bitumi-  
nous, carbonaceous and like materials which 25 comprises mixing with the material to be briquetted a binder including at least two binding materials of different binding ca-  
pacities ground to colloidal fineness, the ground particles of which being capable of 30 remaining in substantially permanent sus-  
pension in water.

4. A process for briquetting coal, peat and like material which comprises mixing with the material to be briquetted a binder 35 formed of at least one of said materials having its original non-colloidal parts ground to colloidal fineness, the ground par-  
ticles being capable of remaining in sub-  
stantially permanent suspension in water.

PETER JUNG.